# EUROPEAN PATENT SPECIFICATION

(11) **EP 3 486 340 B1**
(45) Date of publication and mention of the grant of the patent: **27.01.2021**
(21) Application number: 17827456.9
(22) Date of filing: 30.06.2017
(51) Int. Cl.: C22C 21/00, C22F 1/04, C22F 1/00

(54) **ALUMINUM ALLOY PLASTIC WORKING MATERIAL AND PRODUCTION METHOD THEREFOR**
ALUMINIUMLEGIERUNG-KUNSTSTOFF-ARBEITSMATERIAL UND HERSTELLUNGSVERFAHREN DAFÜR
MATÉRIAU DE TRAVAIL DE MATIÈRE PLASTIQUE ET D'ALLIAGE D'ALUMINIUM ET SON PROCÉDÉ DE PRODUCTION

(30) Priority: 12.07.2016 JP 2016137522
(43) Date of publication of application: 22.05.2019
(73) Proprietor: Nippon Light Metal Company, Ltd., Tokyo 140-8628 (JP)
(72) Inventor: YU Jun, Shizuoka-shi Shizuoka 421-3203 (JP); ISHIWATA Yasuo, Shizuoka-shi Shizuoka 421-3203 (JP); SHIMOSAKA Daisuke, Shizuoka-shi Shizuoka 421-3203 (JP); KONDO Takutoshi, Niigata-shi Niigata 950-3101 (JP); TAGUCHI Yoshihiro, Shizuoka-shi Shizuoka 421-3203 (JP)
(74) Representative: Mewburn Ellis LLP
(86) International application number: PCT/JP2017/024184
(87) International publication number: WO 2018/012326

(56) References cited:
- EP-A1- 2 189 548
- WO-A1-2009/035029
- JP-A- 2010 126 740
- JP-A- 2010 126 740
- JP-A- 2011 105 982
- PELLEGRINI, G ET AL.: 'Growth and Crystallography of the Unidirectionally Solidified Al-Al4Ca Eutectic' MATERIALS SCIENCE AND ENGINEERING vol. 34, February 1978, pages 171 - 181, XP024084573

## Description

### FIELD OF THE INVENTION

The present invention relates to an aluminum alloy plastic working material which has a low Young's modulus, but has an excellent proof stress, and relates to a method for producing the working material.

Since aluminum has many excellent characteristics such as corrosion resistance, electric conductivity, thermal conductivity, light weight, brightness and machinability, aluminum is used for various purposes. In addition, since plastic deformation resistance is small, various shapes can be imparted, and aluminum is also widely used for members subjected to plastic working such as bending processing.

Here, when the rigidity of the aluminum alloy is high, there is a problem that the spring back amount increases when the plastic working such as bending processing is performed, and thus it is difficult to obtain dimensional accuracy. Under such circumstances, an aluminum alloy material having a low Young's modulus is desired, and a method for lowering the Young's modulus of the aluminum alloy material has been studied.

For example, JP 2011-105982 A proposes an aluminum alloy containing an Al phase and an Al₄Ca phase, wherein the Al₄Ca phase contains an Al₄Ca crystallized product, and an average value of the longer side of the Al₄Ca crystallized product is 50 µm or less.

In the aluminum alloy disclosed in JP 2011-105982 A, the movement of the Al₄Ca crystallized product accompanying the dislocation in the matrix becomes easy, so that the rolling workability of the aluminum alloy can be remarkably improved.

### CITATION LIST

### Patent Literature

JP 2011-105982 A is discussed above. EP A 2189548 proposes an aluminum alloy including 0.1 to 12 et% of Ca.

### SUMMARY OF INVENTION

### Technical Problem

However, as represented by, for example, terminals of electrical equipment, the requirement for the dimensional accuracy of the product where aluminum alloys are used has been strict year by year, so that aluminum alloys with lower rigidity are required while maintaining proof stress. Under such technical background, the current situation is that the aluminum alloy of Patent Literature 1 cannot sufficiently satisfy the above requirements.

Considering the above problems in the prior arts, an object of the present invention is to provide an aluminum alloy plastic working material which has a low Young's modulus, but has an excellent proof stress, and relates to a method for efficiently producing the working material.

### Solution to Problem

As a result of extensive study with respect to the aluminum alloy plastic working material and production method therefor in order to achieve the above object, the present inventors have found that it is extremely effective that an Al₄Ca phase is used as the dispersed phase and the crystal structure of the Al₄Ca phase is appropriately controlled, and have reached the present invention.

Namely, a first aspect of the present invention provides an aluminum alloy plastic working material according to claim 1.

By addition of Ca, a compound of Al₄Ca is prepared, which has an activity to lower the Young's modulus of the aluminum alloy. The effect becomes remarkable when the content of Ca is 5.0% or more. To the contrary, when added in excess of 10.0%, the casting property decreases, and since particularly casting by continuous casting such as DC casting becomes difficult, it is necessary to produce by a method with a high production cost such as powder metallurgy method. In the case of producing by the powder metallurgy method, there is a risk that oxides formed on the surface of the alloy powder may get mixed in the product, which may lower the proof stress.

In the aluminum alloy plastic working product of the present invention, though the crystal structure of the Al₄Ca phase which is used as the dispersed phase is basically a tetragonal crystal, the present inventors have intensively studied and found that when the crystal structure of the Al₄Ca phase contains a monoclinic crystal, the proof stress do not decrease so much, but the Young's modulus is greatly decreased. Here, when the intensity ratio (I₁/I₂) of the highest diffraction peak (I₁) attributed to the tetragonal system to the highest diffraction peak (I₂) attributed to the monoclinic system, which are obtained by an X-ray diffraction measurement, is 1 or less, the Young's modulus can be greatly lowered while maintaining the proof stress.

Further, it is preferable that the aluminum alloy plastically working material of the present invention further contains at least one or more of Fe: 0.05 to 1.0 wt% and Ti: 0.005 to 0.05 wt%.

When Fe is contained in the aluminum alloy, the casting property can be improved by broadening the solidification temperature range (solid-liquid coexisting region), and thus the casting surface of the ingot can also be improved. Further there is an effect that the dispersed crystallized product of Fe makes the eutectic structure uniform. The effect becomes remarkable when the Fe content is 0.05 wt% or more. To the contrary, when contained in excess of 1.0 wt%, the eutectic structure becomes coarse and there is a risk to lower the proof stress.

Ti acts as a refining material of the casted structure and exhibits an action to improve casting property, extrudability, and rolling property. The effect is remarkable when the Ti content is 0.005 wt% or more. To the contrary, even when added in excess of 0.05 wt%, it cannot be expected to increase the effect of refining the casted structure, and on the contrary, there is a risk that a coarse intermetallic compound which is to be the starting point of fracture may be generated. It is preferable that Ti is added by a rod hardener (Al-Ti-B alloy) during the casting. B added at this time together with Ti as the rod hardener is acceptable.

Further, in the aluminum alloy plastic working product of the present invention, an average crystal grain size of the Al₄Ca phase is 1.5 µm or less. When the average grain size of the Al₄Ca phase becomes too large, the proof stress of the aluminum alloy decreases, but when the average grain size is 1.5 µm or less, it is possible to suppress the decrease of the proof stress.

Further, a second aspect of the present invention provides a method for producing an aluminum alloy plastic working material according to claim 2.

After the first step for obtaining a plastic workpiece of an aluminum alloy by subjecting an aluminum alloy ingot which contains 5.0 to 10.0 wt% of Ca with the remainder aluminum and inevitable impurities, and has a volume ratio of an Al₄Ca phase which is a dispersed phase of 25% or more to a plastic processing, by conducting the step for subjecting to a heat treatment in a temperature range of 100 to 300 °C (Second step), a part of the tetragonal Al₄Ca phase can be changed into monoclinic crystal.

When the holding temperature in the second step is less than 100 °C, a change from a tetragonal to a monoclinic crystal is difficult to occur, and when the holding temperature is 300 °C or more, recrystallization of the aluminum base material occurs and there is a risk that the proof stress will be lowered. The more preferable temperature range of the heat treatment is 160 to 240 °C. Though the appropriate time for the heat treatment varies depending on the size and shape of the aluminum alloy material, it is preferable that the temperature of the aluminum alloy material itself is kept at least at the holding temperature for 1 hour or more.

In the method for producing the aluminum alloy plastic working material of the present invention, it is preferable that the aluminum alloy ingot contains at least one or more of Fe: 0.05 to 1.0 wt% and Ti: 0.005 to 0.05 wt%.

When Fe is contained in the aluminum alloy, the casting property can be improved by broadening the solidification temperature range (solid-liquid coexisting region), and thus the casting surface of the ingot can also be improved. Further there is an effect that the dispersed crystallized product of Fe makes the eutectic structure uniform. The effect becomes remarkable when the Fe content is 0.05 wt% or more. To the contrary, when contained in excess of 1.0 wt%, the eutectic structure becomes coarse and there is a risk to lower the proof stress.

Ti acts as a refining material of the casted structure and exhibits an action to improve casting property, extrudability, and rolling property. The effect is remarkable when the Ti content is 0.005 wt% or more. To the contrary, even when added in excess of 0.05 wt%, it cannot be expected to increase the effect of refining the casted structure, and on the contrary, there is a risk that a coarse intermetallic compound which is to be the starting point of fracture may be generated. It is preferable that Ti is added by a rod hardener (Al-Ti-B alloy) during the casting. B added at this time together with Ti as the rod hardener is acceptable.

Furthermore, in the method for producing an aluminum alloy plastic working material according to the present invention, it is preferable that, before the first step, the aluminum alloy ingot is not subjected to a heat treatment where the ingot is maintained at a temperature of 400 °C or more.

Generally, in the case of preparing an aluminum alloy, before the ingot is subjected to plastic working, a homogenization treatment is carried out where the ingot is held at a temperature of 400 to 600 °C, but when this homogenization treatment is performed, the Al₄Ca phase contained in the aluminum alloy tends to be large, and the average grain size becomes larger than 1.5 µm. Since the proof stress reduces due to the increase in the average grain size, it is preferable that the homogenization treatment at a holding temperature of 400 °C or higher would not be performed.

### Effects of the invention

According to the present invention, it is possible to provide an aluminum alloy plastic working material which has both an excellent proof stress and a low Young's modulus, and a method for efficiently producing the working material.

### BRIEF DESCRIPTION OF THE DRAWINGS

FIG. 1 is a process chart relating to the method of producing the aluminum alloy plastic working material of the present invention.
FIG. 2 is an X-ray diffraction pattern of the aluminum alloy plastic working material.
FIG. 3 is a photograph of the structure of the present aluminum alloy plastic working material 3.
FIG. 4 is a photograph of the structure of the comparative aluminum alloy plastic working material 3.

### Embodiments for achieving the invention

Hereinafter, the aluminum alloy plastic working material and the method for producing therefor of the present invention will be described in detail with reference to the drawings, but the present inventions are not limited to only those.

### 1. Aluminum alloy plastically working material

### (1) Composition

The aluminum alloy plastic working material includes 5.0 to 10.0 wt% of Ca, and the remainder aluminum and unavoidable impurities. In addition, it is preferable to further contain at least one or more of Fe: 0.05 to 1.0 wt% and Ti: 0.005 to 0.05 wt%.

Each component element will be explained below.

### Ca: 5.0 to 10.0 wt% (preferably 6.0 to 8.0 wt%)

Ca forms a compound of Al₄Ca and has the activity to lower the Young's modulus of the aluminum alloy. The effect becomes remarkable when the content of Ca is 5.0% or more. To the contrary, when added in excess of 10.0%, the casting property decreases, and since particularly casting by continuous casting such as DC casting becomes difficult, it is necessary to produce by a method with a high production cost such as powder metallurgy method. In the case of producing by the powder metallurgy method, there is a risk that oxides formed on the surface of the alloy powder may get mixed in the product, which may lower the proof stress.

### Fe: 0.05 to 1.0 wt%

When Fe is contained, the casting property can be improved by broadening the solidification temperature range (solid-liquid coexisting region), and thus the casting surface of the ingot can also be improved. Further there is an effect that the dispersed crystallized product of Fe makes the eutectic structure uniform. The effect becomes remarkable when being 0.05 wt% or more, and to the contrary, when contained in excess of 1.0 wt%, the eutectic structure becomes coarse and there is a risk to lower the proof stress.

### Ti: 0.005 to 0.05 wt%

Ti acts as a refining material of the casted structure and exhibits an action to improve casting property, extrudability, and rolling property. The effect is remarkable when being 0.005 wt% or more, and to the contrary, even when added in excess of 0.05 wt%, it cannot be expected to increase the effect of refining the casted structure, and on the contrary, there is a risk that a coarse intermetallic compound which is to be the starting point of fracture may be generated. It is preferable that Ti is added by a rod hardener (Al-Ti-B alloy) during the casting. B added at this time together with Ti as the rod hardener is acceptable.

### Other Component Elements

As long as the effects of the present invention are not impaired, it is permissible to contain other elements.

### (2) Structure

The aluminum alloy plastic working material has a volume ratio of an Al₄Ca phase, which is a dispersed phase, is 25% or more, the Al₄Ca phase comprises a tetragonal Al₄Ca phase and a monoclinic Al₄Ca phase, and an intensity ratio (I₁/I₂) of the highest diffraction peak (I₁) attributed to the tetragonal system to the highest diffraction peak (I₂) attributed to the monoclinic system, which are obtained by an X-ray diffraction measurement, is 1 or less.

The tetragonal Al₄Ca phase and the monoclinic Al₄Ca phase exist in the Al₄Ca phase, which is a dispersed phase, and the volume ratio of the combined Al₄Ca phase is 25% or more. By making the volume ratio of the Al₄Ca phase to 25% or more, it is possible to impart an excellent proof stress to the aluminum alloy plastic working material.

Further, an average crystal grain size of the Al₄Ca phase is 1.5 µm or less. When the average grain size of the Al₄Ca phase exceeds 1.5 µm, there is a risk that the proof stress of the aluminum alloy plastic working material decreases.

Though the crystal structure of the Al₄Ca phase is generally a tetragonal crystal, the present inventors have intensively studied and found that when the monoclinic crystal structure exists in the Al₄Ca phase, the proof stress do not almost decrease, but the Young's modulus is greatly decreased. It is not necessary that all crystal structure of the Al₄Ca phases is monoclinic, and it may be in the state of being mixed with the tetragonal crystal. The existence of the Al₄Ca phase which has the monoclinic crystal structure can be identified, for example, by measuring the diffraction peak with X ray diffraction method.

Regarding the Al₄Ca phases, the intensity ratio (I₁/I₂) of the highest diffraction peak (I₁) attributed to the tetragonal system to the highest diffraction peak (I₂) attributed to the monoclinic system, can generally be obtained by a X-ray diffraction measurement. The lattice constants of the tetragonal Al₄Ca are a = 0.4354 and c = 1.118, and the lattice constants of the orthorhombic Al₄Ca are a = 0.6158, b = 0.6175, c = 1.118, β = 88.9 °.

### 2. Method for Producing Aluminum Alloy Plastic Material

FIG. 1 shows a process chart of the aluminum alloy plastic working material of the present invention. The method for producing the aluminum alloy plastic working material of the present invention includes a first step (S01) of subjecting an aluminum alloy ingot to plastic working, and a second step (S02) of applying a heat treatment. Each step and the like will be explained herein below.

### (1) Casting

After subjecting the aluminum alloy molten metal having the composition of the above-mentioned aluminum alloy plastic working material of the present invention to conventionally known molten metal cleaning treatments such as desulfurization treatment, degassing treatment, and filtration treatment, the molten metal is casted into an ingot having a desired shape.

There is no particular restriction on the casting method, and various conventionally known casting methods can be used. For example, it is preferable, by using a continuous casting method such as DC casting, to cast into a shape that the plastic working (extrusion, rolling, forging, etc.) in the first step (S01) is easy to be performed. In the casting, a rod hardener (Al-Ti-B) may be added to improve casting property.

Generally, in the case of preparing an aluminum alloy, before the ingot is subjected to plastic working, a homogenization treatment is carried out where the ingot is held at a temperature of 400 to 600 °C, but when this homogenization treatment is performed, the Al₄Ca phase tends to be large (average grain size of 1.5 µm or larger), and since the proof stress of the aluminum alloy reduces, it is preferable that the homogenization treatment would not be performed in the method for producing aluminum alloy plastic working material according to the present invention.

### (2) First Step (S01)

The first step (S01) is a step of subjecting the aluminum alloy ingot obtained in (1) to the plastic working to obtain a desired shape.

For the plastic working such as extrusion, rolling, or forging, either hot working or cold working may be used, or a plurality of them may be combined. By performing the plastic working, the aluminum alloy becomes a processed structure, and the proof stress is improved. In the stage of the plastic working, most Al₄Ca phases contained in the aluminum alloy have the tetragonal crystal structure.

### (3) Second Step (S02)

The second step (S02) is a step for applying the heat treatment to the aluminum alloy plastic working material obtained in the first step (S01).

By subjecting the aluminum alloy plastic working material subjected to plastic working in the first step (S01) to the heat treatment at 100 to 300 °C, a part of the tetragonal Al₄Ca phase can be converted into the monoclinic crystal. The change from the tetragonal to the monoclinic is difficult to occur when the holding temperature is less than 100 °C. On the other hand, since, when the holding temperature is 300 °C or higher, recrystallization of the aluminum base material may occur and there is a risk that the proof stress may be reduced, the holding temperature of the heat treatment is preferably 100 to 300 °C, more preferably 160 to 240 °C.

Though the optimum period of time for the heat treatment varies depending on the size and shape of the aluminum alloy plastic working material to be treated, it is preferable that the temperature of at least the aluminum alloy plastic working material is kept at the above holding temperature for 1 hour or more.

The representative embodiments of the present invention have been described above, but the present invention is not limited only to these embodiments, and various design changes are possible, and all such design changes are included in the technical scope of the present invention.

### EXAMPLES

### <<Example>>

An aluminum alloy having the composition shown Table 1 was cast into an ingot (billet) of ϕ8 inches by a DC casting method without any homogenization treatment, and then, plastic-working at an extrusion temperature of 500 °C to obtain a plate having a width of 180 mm × a thickness of 8 mm. Then, after cold rolling to a thickness of 5 mm, a heat treatment was carried out to hold at 200 °C for 4 hours to obtain the present aluminum alloy working plastic material.

**[Table 1]**

| (unit: wt%) | | | | |
|---|---|---|---|---|
| | Ca | Fe | Ti | Al |
| Present aluminum alloy plastic working material 1 | 5.2 | 0.001 | 0.002 | Bal. |
| Comparative aluminum alloy plastic working material 1 | | | | |
| Present aluminum alloy plastic working material 2 | 6.2 | 0.05 | 0.002 | Bal. |
| Comparative aluminum alloy plastic working material 2 | | | | |
| Present aluminum alloy plastic working material 3 | 7.3 | 0.05 | 0.01 | Bal. |
| Comparative aluminum alloy plastic working material 3 | | | | |
| Present aluminum alloy plastic working material 4 | 8.1 | 0.001 | 0.01 | Bal. |
| Comparative aluminum alloy plastic working material 4 | | | | |
| Present aluminum alloy plastic working material 5 | 9.5 | 0.05 | 0.05 | Bal. |
| Comparative aluminum alloy plastic working material 5 | | | | |

The obtained present aluminum alloy plastic working material 3 was subjected to the X-ray diffraction measurement to measure the position pf the peak of the Al₄Ca phase. In the X-ray diffraction measurement, a specimen of 20 mm × 20 mm was cut out from the plate-like aluminum alloy plastic working material, the surface layer portion was removed by about 500 µm, and then a θ-2 θ measurement was carried out with respect to the region from a Cu-Ka beam source. The results are shown in FIG. 2. The intensity ratio (I₁/I₂) of the highest diffraction peak (I₁) attributed to the tetragonal system to the highest diffraction peak (I₂) attributed to the monoclinic system was 0.956.

In addition, JIS-14B specimens were cut out from the present aluminum alloy plastic working materials 1 to 5, and the Young's modulus and proof stress were measured by a tensile test. The obtained results are shown in Table 2. In addition, the volume ratio of the dispersed phase (Al₄Ca phase) calculated from the structural observation by the optical microscope are shown in Table 2.

The present aluminum alloy plastic working materials 6 to 9 were obtained in the same manner as in the case of the present aluminum alloy plastic working material 3 except that the heat treatment temperature was any one of 100 °C, 160 °C, 240 °C and 300 °C. In addition, in the same manner as in the case of the present aluminum alloy plastic working materials 1 to 5, the Young's modulus and proof stress were measured by a tensile test. The obtained results are shown in Table 3.

### <<Comparative Example>>

An aluminum alloy having the composition shown Table 1 was cast into an ingot (billet) of ϕ8 inches by a DC casting method without any homogenization treatment, and then, plastic-working at an extrusion temperature of 500 °C to obtain a plate having a width of 180 mm × a thickness of 8 mm. Thereafter, the cold rolling to a thickness of 5 mm was carried out to obtain the comparative aluminum alloy plastic working materials 1 to 5.

The obtained comparative aluminum alloy plastic working material 3 was subjected to the X-ray diffraction measurement to measure the position pf the peak of the Al₄Ca phase. In the X-ray diffraction measurement, a specimen of 20 mm × 20 mm was cut out from the plate-like aluminum alloy plastic working material, the surface layer portion was removed by about 500 µm, and then a θ-2 θ measurement was carried out with respect to the region from a Cu-Kα beam source. The results are shown in FIG. 2. The intensity ratio (I₁/I₂) of the highest diffraction peak (I₁) attributed to the tetragonal system to the highest diffraction peak (I₂) attributed to the monoclinic system was 1.375.

In addition, JIS-14B specimens were cut out from the comparative aluminum alloy plastic working materials 1 to 5, and the Young's modulus and proof stress were measured by a tensile test. The obtained results are shown in Table 2.

The comparative aluminum alloy plastic working materials 6 and 7 were obtained in the same manner as in the case of the present aluminum alloy plastic working material 3 except that the heat treatment temperature was 90 °C and 310 °C. In addition, in the same manner as in the case of the comparative aluminum alloy plastic working materials 1 to 5, the Young's modulus and proof stress were measured by a tensile test. The obtained results are shown in Table 3.

The comparative aluminum alloy plastic working material 8 was obtained in the same manner as in the case of the present aluminum alloy plastic working material 3 except that, after casting in an ingot (billet), the homogenization treatment was carried out while holding at 550 °C. In addition, JIS-14B specimen was cut out from the comparative aluminum alloy plastic working material 8, and the Young's modulus and proof stress were measured by a tensile test. The obtained results are shown in Table 4. The Young's modulus and the proof stress of the present aluminum alloy plastic working material 3 which is different only in the presence or absence of homogenization treatment are also shown as comparison data.

**[Table 2]**

| | Heat treatment | Volume ratio of dispersed phase | Young's modulus | Proof stress | Tensile strength |
|---|---|---|---|---|---|
| | | (%) | (GPa) | (MPa) | (MPa) |
| Present aluminum alloy plastic working material 1 | Did | 26.7 | 58 | 147 | 245 |
| Present aluminum alloy plastic working material 2 | | 31.2 | | 167 | 258 |
| Present aluminum alloy plastic working material 3 | | 35.9 | 53 | 169 | 254 |
| Present aluminum alloy plastic working material 4 | | 39.9 | 51 | 208 | 272 |
| Present aluminum alloy plastic working material 5 | | 44.3 | 48 | 173 | 269 |
| Comparative aluminum alloy plastic working material 1 | Non | - | 67 | 176 | 259 |
| Comparative aluminum alloy plastic working material 2 | | - | 64 | 184 | 268 |
| Comparative aluminum alloy plastic working material 3 | | - | 61 | 189 | 265 |
| Comparative aluminum alloy plastic working material 4 | | - | 57 | 222 | 285 |
| Comparative aluminum alloy plastic working material 5 | | - | 56 | 186 | 276 |

From the results shown in Table 2, when comparing the present aluminum alloy plastic working material having the same composition with the comparative aluminum alloy plastic working material, the Young's modulus of the aluminum alloy plastic working materials of the present invention (the present aluminum alloy plastic working materials 1 to 5) are greatly lower than the Young's modulus of the comparative aluminum alloy plastic working materials 1 to 5 which were not subjected to the heat treatment. On the other hand, the proof stress and tensile strength of the present aluminum alloy plastic working materials 1 to 5 are not greatly reduced as compared with the comparative aluminum alloy plastic working materials 1 to 5. It is clear that the volume ratios of the dispersed phase (Al₄Ca phase) in the aluminum alloy plastic working materials of the present invention are 25% or more.

**[Table 3]**

| | Heat treatment temperature | Young's modulus | Proof stress | Tensile strength |
|---|---|---|---|---|
| | (°C) | (GPa) | (MPa) | (MPa) |
| Present aluminum alloy plastic working material 6 | 100 | 54 | 187 | 267 |
| Present aluminum alloy plastic working material 7 | 160 | 54 | 172 | 262 |
| Present aluminum alloy plastic working material 8 | 240 | 53 | 167 | 252 |
| Present aluminum alloy plastic working material 9 | 300 | 52 | 161 | 240 |
| Comparative aluminum alloy plastic working material 6 | 90 | 59 | 195 | 275 |
| Comparative aluminum alloy plastic working material 7 | 310 | 53 | 143 | 231 |

From the results shown in Table 3, when the holding temperature of the heat treatment is 90 °C (comparative aluminum alloy plastic working material 6), the Young's modulus shows a high value (almost not lowered). In addition, when the holding temperature of the heat treatment is 310 °C (comparative aluminum alloy plastic working material 7), though the Young's modulus is lowered, the proof stress and tensile strength are simultaneously lowered. From the results, when the holding temperature of the heat treatment was 310 °C, it is considered that the recrystallization of the plastic working structure progressed.

The structural photographs of the present aluminum alloy plastic working material 3 and the comparative aluminum alloy plastic working material 8 by an optical microscope are shown in FIG. 3 and FIG. 4, respectively. In the structure photograph, the black region is the Al₄Ca phase, and the average crystal grain size of the Al₄Ca phase is measured by image analysis. The obtained results are shown in Table 4.

**[Table 4**

| | Homogenization treatment | Average crystal grain size of Al₄Ca phase | Young's modulus | Proof stress | Tensile strength |
|---|---|---|---|---|---|
| | | (µm) | (GPa) | (MPa) | (MPa) |
| Comparative aluminum alloy plastic working material 8 | Did | 1.56 | 53 | 158 | 229 |
| Present aluminum alloy plastic working material 3 | Non | 1.15 | 53 | 169 | 254 |

From the results shown in Table 4, when subjecting to the homogenization treatment maintained at 550 °C (comparative aluminum alloy plastic working material 8), it is recognized that the proof stress and the tensile strength are reduced. Here, the average crystal grain size of the Al₄Ca phase is increased by the homogenization treatment to 1.56 µm. It is considered that the proof stress and the tensile strength are reduced due to the increase in the average crystal grain size.

## Claims

1. An aluminum alloy plastic working material, which comprises:
5.0 to 10.0 wt% of Ca,
optionally at least one or more of 0.05 to 1.0 wt% of Fe and 0.005 to 0.05 wt%. of Ti, and
the remainder aluminum and unavoidable impurities,
wherein:
a volume ratio of an Al₄Ca phase, which is a dispersed phase, is 25% or more,
the Al₄Ca phase comprises a tetragonal Al₄Ca phase and a monoclinic Al₄Ca phase,
an intensity ratio (I₁/I₂) of the highest diffraction peak (I₁) attributed to the tetragonal system to the highest diffraction peak (I₂) attributed to the monoclinic system, which are obtained by an X-ray diffraction measurement, is 1 or less, and
an average crystal grain size of the Al₄Ca phase is 1.5 µm or less.

2. A method for producing an aluminum alloy plastic working material, comprising:
a first step for obtaining a plastic workpiece of an aluminum alloy by subjecting an aluminum alloy ingot which contains 5.0 to 10.0 wt% of Ca and optionally contains at least one or more of 0.05 to 1.0 wt% of Fe and 0.005 to 0.05 wt%. of Ti with the remainder aluminum and inevitable impurities, and has a volume ratio of an Al₄Ca phase which is a dispersed phase of 25% or more to a plastic processing, and
a second step for subjecting to a heat treatment in a temperature range of 100 to 300 °C.

3. The method for producing an aluminum alloy plastic working material according to claim 2, wherein, before the first step, the aluminum alloy ingot is not subjected to a heat treatment where the ingot is maintained at a temperature of 400 °C or more.

## Patentansprüche

1. Plastisches Aluminiumlegierungsarbeitsmaterial, das Folgendes umfasst:
5,0 bis 10,0 Gew.-% Ca,
gegebenenfalls zumindest eines oder mehrere aus 0,05 bis 1,0 Gew.-% Fe und 0,005 bis 0,05 Gew.-% Ti und
den Rest Aluminium und unvermeidbare Verunreinigungen,
wobei:
der Volumenanteil einer Al₄Ca-Phase, die eine dispergierte Phase ist, 25 % oder mehr beträgt,
die Al₄Ca-Phase eine tetragonale Al₄Ca-Phase und eine monokline Al₄Ca-Phase umfasst,
das Intensitätsverhältnis (I₁/I₂) zwischen dem höchsten Beugungsreflex (I1), der dem tetragonalen System zugeordnet ist, und dem höchsten Beugungsreflex (I₂), der dem monoklinen System zugeordnet ist, beide erhalten durch eine Röntenbeugungsmessung, 1 oder weniger beträgt und
die durchschnittliche Kristallkorngröße der Al₄Ca-Phase 1,5 µm oder weniger beträgt.

2. Verfahren zur Herstellung eines plastischen Aluminiumlegierungsarbeitsmaterials, das Folgendes umfasst:
einen ersten Schritt zum Erhalten eines plastischen Werkstücks aus einer Aluminiumlegierung durch Aussetzen des Aluminiumlegierungsblocks, der 5,0 bis 10,0 Gew.-% Ca enthält und gegebenenfalls zumindest eines oder mehrere aus 0,05 bis 1,0 Gew.-% Fe und 0,005 bis 0,05 Gew.-% Ti enthält, wobei der Rest Aluminium und unvermeidbare Verunreinigungen sind, und der einen Volumenanteil einer Al₄Ca-Phase, die eine dispergierte Phase ist, von 25 % oder mehr aufweist, gegenüber einer plastischen Bearbeitung und
einen zweiten Schritt zum Aussetzen gegenüber einer Wärmebehandlung in einem Temperaturbereich von 100 bis 300 °C.

3. Verfahren zur Herstellung eines plastischen Aluminiumlegierungsarbeitsmaterials nach Anspruch 2, wobei der Aluminiumlegierungsblock vor dem ersten Schritt keiner Wärmebehandlung ausgesetzt wird, bei welcher der Block bei einer Temperatur von 400 °C oder mehr gehalten wird.

## Revendications

1. Matériau d'usinage plastique et d'alliage d'aluminium, qui contient :
de 5,0 à 10,0 % en poids de Ca,
facultativement au moins un ou plusieurs parmi 0,05 à 1,0 % en poids de Fe et 0,005 à 0,05 % en poids de Ti, et
le reste étant de l'aluminium et des impuretés inévitables, dans lequel :
un rapport volumique d'une phase Al₄Ca, qui est une phase dispersée, est de 25 % ou plus,
la phase Al₄Ca comprend une phase tétragonale Al₄Ca et une phase monocyclique Al₄Ca,
un rapport d'intensité (I₁/I₂) entre le pic de diffraction le plus élevé (I₁) attribué au système tétragonal et le pic de diffraction le plus élevé (I₂) attribué au système monocyclique, qui sont obtenus par une mesure de diffraction des rayons X, est inférieur ou égal à 1, et
une taille de grain cristallin moyenne de la phase Al₄Ca est de 1,5 µm ou moins.

2. Procédé de production d'un matériau d'usinage plastique d'alliage d'aluminium, comprenant :
une première étape pour obtenir une pièce d'usinage plastique constituée d'un alliage d'aluminium en soumettant un lingot d'alliage d'aluminium qui contient 5,0 à 10,0 % en poids de Ca et contient facultativement au moins un ou plusieurs parmi 0,05 à 1,0 % en poids de Fe et 0,005 à 0,05 % en poids de Ti, le reste étant de de l'aluminium et des impuretés inévitables, et a un rapport volumique d'une phase Al₄Ca qui est une phase dispersée de 25 % ou plus à un traitement plastique, et
une seconde étape de soumission à un traitement thermique dans une plage de température de 100 à 300°C.

3. Procédé de production d'un matériau d'usinage plastique d'alliage d'aluminium selon la revendication 2, dans lequel, avant la première étape, le lingot d'alliage d'aluminium n'est pas soumis à un traitement thermique où le lingot est maintenu à une température de 400°C ou plus.
